# EUROPEAN PATENT SPECIFICATION

(11) **EP 0 804 293 B1**
(45) Date of publication and mention of the grant of the patent: **09.06.1999**
(21) Application number: 95944604.8
(22) Date of filing: 06.12.1995
(51) Int. Cl.: B05D 5/06

(54) **MULTI-COLOR PATTERNED COOKWARE**
VIELFÄRBIG GEMUSTERTES KOCHGESCHIRR
ARTICLE DE CUISSON PRESENTANT UN MOTIF MULTICOLORE

(30) Priority: 22.12.1994 US 362078; 22.12.1994 US 362079; 22.12.1994 US 362090; 07.06.1995 US 476929; 07.06.1995 US 481682; 07.06.1995 US 482373
(43) Date of publication of application: 05.11.1997
(62) Divisional of application: 98203949.7
(73) Proprietor: E.I. DU PONT DE NEMOURS AND COMPANY, Wilmington Delaware 19898 (US)
(72) Inventor: BATZAR, Kenneth, Cherry Hill, NJ 08003-3215 (US); MASON, Lori, Marie, North Wales, PA 19454-4215 (US)
(74) Representative: Matthews, Derek Peter
(86) International application number: US9515793
(87) International publication number: WO9619299

(56) References cited:
- EP-A- 0 022 256
- US-A- 4 259 375
- US-A- 4 353 950
- US-A- 5 240 775
- US-A- 5 250 356

## Description

### BACKGROUND OF THE INVENTION

This invention concerns non-stick coated cookware, with a decorative pattern visible through a light transmitting topcoat. More specifically, it concerns such cookware with a pattern formed by discontinuous globules..

U.S. Patent 4,259,375 - Vassiliou (1981) discloses an article of cookware with a 3-layer coating having a discontinuous speckled or spattered pattern in a partial layer directly beneath the topcoat. The spattered coating is deliberately sprayed directly on the layer under it while the under layer is still wet and soft so that the spattered layer sinks into the under layer and does not provide roughness that could telegraph through the surface. It was said that roughness would provide a place for a fork or other utensil to catch in the coating and tear the coating. The spattered layer dots were also sprayed on directly, such as at 90 degrees from the substrate, so as to form more or less round dots. This patent is incorporated by reference herein for its disclosure of materials, processes and equivalents suitable for the present invention.

U.S. Patent 3,961,993 - Palisin (1976) discloses spraying multilayer polymer coatings on a substrate, one layer being sprayed on top of the layer under it after the under layer has become tacky. A tacky underlayer permits the successive layer to adhere better without completely merging indistinguishably with the underlayer. Still, any roughness in the upper layer would tend to smooth out as the two layers interact.

U.S. Patent 3,655,421 - Long (1972) describes means of keeping globules of an intermittent coating from flowing out to make a uniform layer, by controlling surface tension relations.

It is desirable to have a superior non-stick, decorative coating for cookware optionally with a raised or textured surface and with greater flexibility for aesthetic design than just to make smooth round dots.

### SUMMARY OF THE INVENTION

The present invention provides an article of cookware and a method of making it, having a cooking surface which comprises a multi-layer, non-stick coating on a substrate which coating minimizes sticking by food residues and which is heat resisting by being stable at temperatures above 300° C, wherein the coating comprises a primer adhered to the substrate, a non-stick, heat-resisting, light-transmitting topcoat, and optionally one or more intermediate coats, with the topcoat adhered to any such intermediate coats which are adhered to the primer or, in the absence of intermediate coats, the topcoat being adhered directly to the primer, with the intermediate coat under the topcoat having a first color or darkness or, in the absence of intermediate coats, the primer having a first color or darkness, characterised by spraying at least two applications of globules to form a discontinuous layer on or in and covering no more than 80% of the area of the intermediate coat under the topcoat or, in the absence of intermediate coats, the primer, said globules having at least one color or darkness which is visibly different from said first color or darkness as seen through said topcoat, with the first application covering 30-80% of the area and the second application covering 20-45% of the area, with the second application covering at least 5% less area than the first.

Included in the invention are a method of making an article in which the coatings are applied by spraying coating compositions successively on the substrate and ultimately heating the article to cure the coating, wherein the coating under the discontinuous coating is dried enough before applying the discontinuous coating so that substantial portions of the spattered coating remains on top of said under coating to create the roughness telegraphing through the topcoat. In another alternative the undercoat is not dried before applying the discontinuous coat which then sinks into the undercoat, resulting in a substantially smooth topcoat.

### DETAILED DESCRIPTION

One embodiment of the process for obtaining the present invention is the drying or "flashing" the primer or intermediate coat before applying the discontinuous coat, adequately so the spattered dots do not sink into the primer or the intermediate coat. In normal application, air flow for 30 seconds or longer, or preheating the substrate or the air with a shorter time of air flow, will suffice.

In another embodiment, the globules can be applied wet-on-wet and permitted to sink into the underlayer so long as they do not merge and lose their distinctiveness.

Those skilled in the art know how to select the ingredients of each coating to avoid wetting which might cause the globules to run together. Wetting is generally not a problem with most heat resistant materials useful for cookware coatings, especially perfluoropolymers such as polytetrafluoroethylene and (PTFE) and copolymers of TFE and fluorovinyl ethers (PFA).

Preferably the coatings contain oxide-coated mica, and preferably the oxide in Ti0₂, as described in U.S. Patents 3,087,827 - Klenke et al., 3,087,828 and 3,087,829 - both to Linton, and granted 1963.

In the examples which follow, parts, percentages and proportions are given by weight except where stated otherwise.

### EXAMPLE 1

A primer having the composition of Table 1 is sprayed on a clean, lightly etched aluminum substrate to a dry film thickness (DFT) of 7.5 to 10 microns, the primer is dried at 66°C for 3 minutes and a black midcoat of Table 2 is applied to a DFT of 17.5 to 20 microns. The midcoat is allowed to dry at ambient temperature for 45 seconds and three separate inks or spatter coatings are applied using a DeVilbiss spatter gun to provide a discontinuous coating. The inks of Table 3 or 4 are colored to be significantly different than the black midcoat background and are sprayed at a 45° angle (or at an angle of from 30 to 75°) to provide irregular shapes on the spinning substrate. The effect is to provide an appearance of natural stone. The inks are not limited to solid color pigments but also include color achieved by reflectance with coated mica. A topcoat of Table 5 is then applied wet-on-wet over the spattered particles. The topcoat, in this example, contains mica particles in a 1-15 micron particle size range so as not to interfere with the aesthetics of the spatter coat. The entire system is sintered at 427 to 435°C for 5 minutes with the measured temperatures being that of the substrate metal.

**TABLE 1**

| Primer | Coating Composition (Wt. %) | Solids Content in Finished Article (Wt%) |
|---|---|---|
| Furfuryl Alcohol | 1.82 | - |
| Polyamic acid salt in N-Methyl Pyrrolidone | 18.10 | 24.48 |
| Water | 48.33 | - |
| Mica coated with TiO₂ | 0.05 | 0.24 |
| PTFE Dispersion | 7.93 | 22.19 |
| FEP Dispersion | 5.88 | 15.08 |
| Colloidal Silica Dispersion | 3.58 | 5.00 |
| Ultramarine blue dispersion | 13.74 | 32.06 |
| Aluminum silicate dispersion | 0.58 | 0.94 |

**TABLE 2**

| Intermediate | Coating Composition (Wt. %) | Solids Content in Finished Article (Wt%) |
|---|---|---|
| PTFE Dispersion | 56.34 | 77.43 |
| PFA Dispersion | 10.21 | 14.22 |
| Water | 4.62 | - |
| Carbon black dispersion | 2.71 | 3.79 |
| Ultramarine blue dispersion | 0.49 | 3.22 |
| Mica coated with TiO₂ | 0.75 | 1.73 |
| Surfactant catalyst soln. | 12.63 | - |
| Acrylic dispersion | 12.23 | - |

**TABLE 3**

| Typical spatter ink formulation compositions (parts by weight) | | | |
|---|---|---|---|
| | A (white) | B (gray) | C (brown) |
| PTFE Dispersion | 542.0 | 542.0 | 542.0 |
| PFA Dispersion | 96.0 | 96.0 | 96.0 |
| Ceramic Dispersion | 50.0 | 50.0 | - |
| TiO₂ Dispersion | 100.0 | 100.0 | 20.0 |
| Iron Oxide Dispersion | - | - | 80.00 |
| Channel Black Dispersion | - | 8.0 | 2.0 |
| Solvent Surfactant Blend | 110.00 | 110.00 | 110.00 |
| Acrylic Dispersion | 120.00 | 120.00 | 120.00 |
| Solvent-Surfactant Blend | 30.00 | 30.00 | 30.00 |
| Hydroxyl propl cellulose soln. | 30.00 | 15.00 | 20.00 |
| Viscosity in centipoise as measured by Brookfield #2 spindle, @ 20 rpm | 682 | 608 | 682 |

**TABLE 4**

| | White | | Grey | |
|---|---|---|---|---|
| Spatter Coats | Coating Composition (Wt. %) | Solids Content in Finished Article (Wt. %) | Coating Composition (Wt. %) | Solids Content in Finishes Article (Wt. %) |
| PTFE Dispersion | 50.29 | 71.04 | 50.61 | 70.63 |
| PFA Dispersion | 8.91 | 12.58 | 8.96 | 12.52 |
| Al₂O₃ Ceramic Dispersion | 4.64 | 5.46 | 4.67 | 5.43 |
| TiO₂ Dispersion | 9.28 | 10.92 | 9.34 | 10.86 |
| Carbon black Dispersion | - | - | 0.75 | 0.52 |
| Surfactant-Catalyst Solution | 12.99 | - | 13.07 | - |
| Acrylic Dispersion | 11.13 | - | 11.20 | - |
| Hydroxyl propyl cellulose solution | 2.78 | - | 1.40 | - |
| Viscosity in centipoise as measured by Brookfield #2 spindle, @ 20 rpm | 682 | | 608 | |

**TABLE 5**

| Topcoat | Coating Composition (Wt. %) | Solids Content in Finished Article (Wt%) |
|---|---|---|
| PTFE Dispersion | 66.73 | 94.04 |
| PFA Dispersion | 3.51 | 4.95 |
| Water | 3.77 | - |
| Mica coated with TiO₂ | 0.43 | 1.01 |
| Surfactant catalyst soln. | 12.52 | - |
| Acrylic dispersion | 13.04 | - |

In order to achieve a stone-like appearance, we prefer to spray a first discontinuous coat of a relatively darker color or optical density than the second as well as each successive globule coat being of a progressively lighter color or darkness. One preferred combination is to have a black base coat (the intermediate on which the discontinuous globule coats are to be sprayed) with the first globule coat in a dark brown, the second globule coat in a lighter gray, and an optional third globule coat in white.

It is important, for achieving the desired aesthetic flexibility, to have more complete coverage with the first globule coat and progressively less complete coverage with each successive globule coat, in accordance with the following:

**TABLE 6**

| | % of Area | |
|---|---|---|
| Globule Coat | Range of Coverage | Preferred Range |
| First | 30-80 | 45-65 |
| Second | 20-45 | 30-40 |
| Optional Third | 10-35 | 15-30 |

There should be at least a 5% difference in area covered between each globule coat. Thus, if the first coat covers 40%, the second should cover no more than 35% and then the third no more than 30%.

The spray is preferably done from a spatter gun, resulting in random coverage and more or less overlap of the globules of one application by those of the next application.

## Claims

1. A method of making an article of cookware having a cooking surface which comprises a multi-layer, non-stick coating on a substrate which coating minimizes sticking by food residues and which is heat resisting by being stable at temperatures above 300°C, wherein the multi-layer coating comprises: (1) a primer adhered to the substrate, (2) a non-stick, heat-resisting, light-transmitting topcoat, and (3) optionally one or more intermediate coats, with the topcoat adhered to any such intermediate coats which are adhered to the primer or, in the absence of intermediate coats, the topcoat being adhered directly to the primer, with the intermediate coat under the topcoat having a first color or darkness or, in the absence of intermediate coats, the primer having a first color or darkness, characterised by spraying at least two applications of globules to form a discontinuous layer on or in and covering no more than 80% of the area of the intermediate coat under the topcoat or, in the absence of intermediate coats, the primer, said globules having at least one color or darkness which is visibly different from said first color or darkness as seen through said topcoat, with the first application covering 30-80% of the area and the second application covering 20-45% of the area, with the second application covering at least 5% less area than the first.

2. The method of claim 1 wherein a third application is made to a coverage of 10-35%, with the third application covering at least 5% less area than the second.

3. The method of claim 1 wherein the first application coverage is in the range of 45-65% and the second application coverage is in the range of 30-40%.

4. The method of claim 3 wherein the third application coverage is in the range of 15-30%.

5. A method according to any of claims 1 to 4 wherein the discontinuous layer is sprayed on the coating under it while said undercoating is partially dried prior to applying the discontinuous coating so as to create a texture of roughness in the topcoat.

6. A method according to any of claims 1 to 4 wherein the discontinuous layer is sprayed on the coating under it while said under coating is still wet enough so that the globules sink into said undercoating and the final topcoat is substantially smooth.

7. A method according to any of claims 1 to 6 wherein the discontinuous layer is sprayed onto the undercoating on the substrate at an angle of the center of the spray stream to the substrate in the range of 30 to 75 degrees creating a splattered coating of non-round dots.

8. The method of claim 7 wherein the angle is in the range of 45 to 60 degrees.

9. The method of claim 8 wherein each successive globule application is of a lighter color or darkness than the layer beneath it.

10. An article of cookware made by any of the methods of claims 1 to 9.

## Patentansprüche

1. Verfahren zur Herstellung eines Kochgeschirr-Gegenstands mit einer Kochoberfläche, welche eine mehrschichtige Antikleb-Beschichtung auf einem Substrat umfaßt, wobei die Beschichtung das Kleben von Lebensmittelrückständen minimiert und wärmebeständig ist, indem sie bei Temperaturen oberhalb von 300° C stabil ist, wobei die mehrschichtige Beschichtung umfaßt: (1) einen an dem Substrat haftenden Primer, (2) einen wärmebeständigen, lichtdurchlässigen Antikleb-Decküberzug und (3) gegebenenfalls einen oder mehrere Zwischenüberzüge, wobei der Decküberzug an jeglichen derartigen Zwischenüberzügen, die an dem Primer haften, haftet, oder der Decküberzug in Abwesenheit von Zwischenüberzügen direkt am Primer haftet, wobei der Zwischenüberzug unter dem Decküberzug eine erste Farbe oder Dunkelheit aufweist, oder, in der Abwesenheit von Zwischenüberzügen, der Primer eine erste Farbe oder Dunkelheit aufweist, gekennzeichnet durch das Sprühen von mindestens zwei Anwendungen von Kügelchen unter Bildung einer diskontinuierlichen Schicht auf oder in der Fläche des Zwischenüberzugs unter dem Decküberzug oder, in Abwesenheit von Zwischenüberzügen, des Primers, die nicht mehr als 80% derselben bedeckt, wobei die Kügelchen mindestens eine Farbe oder Dunkelheit aufweisen, die sich sichtbar von der ersten Farbe oder Dunkelheit unterscheidet, wie durch den Decküberzug betrachtet, wobei die erste Anwendung 30 - 80% der Fläche bedeckt und die zweite Anwendung 20 - 45% der Fläche bedeckt, wobei die zweite Anwendung mindestens 5% weniger Fläche als die erste bedeckt.

2. Verfahren nach Anspruch 1, in welchem eine dritte Anwendung mit einer Bedeckung von 10 - 35% durchgeführt wird, wobei die dritte Anwendung mindestens 5% weniger Fläche als die zweite bedeckt.

3. Verfahren nach Anspruch 1, in welchem die erste Anwendungsbedeckung im Bereich von 45 - 65% liegt und die zweite Anwendungsbedeckung im Bereich von 30 - 40% liegt.

4. Verfahren nach Anspruch 3, in welchem die dritte Anwendungsbedeckung im Bereich von 15 - 30% liegt.

5. Verfahren nach irgendeinem der Ansprüche 1 bis 4, in welchem die diskontinuierliche Schicht auf die Beschichtung unter derselben gesprüht wird, wahrend die Unterbeschichtung vor der Aufbringung der diskontinuierlichen Beschichtung teilweise getrocknet ist, um eine Textur oder Rauheit in dem Decküberzug zu erzeugen.

6. Verfahren nach irgendeinem der Ansprüche 1 bis 4, in welchem die diskontinuierliche Schicht auf die Beschichtung unter derselben gesprüht wird, während die Unterbeschichtung noch naß genug ist, daß die Kügelchen in die Unterbeschichtung einsinken und der endgültige Decküberzug im wesentlichen glatt ist.

7. Verfahren nach irgendeinem der Ansprüche 1 bis 6, in welchem die diskontinuierliche Schicht auf die Unterbeschichtung auf dem Substrat in einem Winkel des Mittelpunkts des Sprühstroms zum Substrat im Bereich von 30 bis 75° aufgesprüht wird, was eine gesprenkelte Beschichtung von unrunden Pünktchen erzeugt.

8. Verfahren nach Anspruch 7, in welchem der Winkel im Bereich von 45 bis 60° liegt.

9. Verfahren nach Anspruch 8, in welchem jede aufeinanderfolgende Kügelchen-Anwendung von hellerer Farbe oder Dunkelheit als die Schicht darunter ist.

10. Kochgeschirr-Gegenstand, hergestellt nach irgendeinem der Verfahren nach den Ansprüchen 1 bis 9.

## Revendications

1. Procédé de fabrication d'un article de cuisson possédant une surface de cuisson qui comprend un revêtement antiadhésif multicouche sur un substrat, lequel revêtement minimise l'adhérence des résidus de nourriture et qui est résistant à la chaleur en étant stable à des températures supérieures à 300°C, le revêtement multicouche comprenant : (1) une couche de fond collée au substrat, (2) une couche de finition antiadhésive transparente résistant à la chaleur, et (3) facultativement une ou plusieurs couches intermédiaires, la couche de finition collant à n'importe laquelle de ces couches intermédiaires qui sont collées sur la couche de fond ou, en l'absence de couches intermédiaires, la couche de finition étant collée directement sur la couche de fond, la couche intermédiaire sous la couche de finition ayant une première couleur ou teinte foncée, ou en l'absence de couches intermédiaires, la couche de fond ayant une première couleur ou teinte foncée, caractérisé en ce qu'au moins deux applications de globules sont pulvérisées pour former une couche discontinue sur ou dans et recouvrant 80% au maximum de la surface de la couche intermédiaire sous la couche de finition, ou en l'absence de couches intermédiaires, la couche de fond, lesdits globules ayant au moins une couleur ou teinte foncée, qui est visiblement différente de ladite première couleur ou teinte foncée telle que vue au travers de ladite couche de finition, la première application couvrant 30 à 80% de la surface et la deuxième application couvrant 20 à 45% de la surface, la deuxième application couvrant au moins 5% de surface en moins que la première.

2. Procédé suivant la revendication 1, dans lequel une troisième application couvre 10 à 35%, la troisième application couvrant au moins 5% de surface en moins que la seconde.

3. Procédé suivant la revendication 1, dans lequel la première application couvre 45 à 65%, la seconde application couvrant 30 à 40%.

4. Procédé suivant la revendication 3, dans lequel la troisième application couvre 15 à 30%.

5. Procédé suivant l'une quelconque des revendications 1 à 4, dans lequel la couche discontinue est pulvérisée sur le revêtement situé en dessous d'elle tandis que ledit revêtement du dessous est partiellement séché avant d'appliquer le revêtement discontinu de façon à créer une texture de rugosité dans la couche de finition.

6. Procédé suivant l'une quelconque des revendications 1 à 4, dans lequel la couche discontinue est pulvérisée sur le revêtement situé en dessous d'elle tandis que ledit revêtement du dessous est encore suffisamment humide pour que les globules s'enfoncent dans ledit revêtement du dessous et la couche de finition finale est pratiquement lisse.

7. Procédé suivant l'une quelconque des revendications 1 à 6, dans lequel la couche discontinue est pulvérisée sur le revêtement du dessous sur le substrat sous un angle du centre de la pulvérisation vers le substrat dans l'intervalle de 30 à 75 degrés, créant un revêtement irrégulier de points non ronds.

8. Procédé suivant la revendication 7, dans lequel l'angle est dans l'intervalle de 45 à 60 degrés.

9. Procédé suivant la revendication 8, dans lequel chaque application successive de globules est d'une couleur ou teinte foncée, plus claire que la couche située en dessous d'elle.

10. Article de cuisson fabriqué suivant l'un quelconque des procédés des revendications 1 à 9.
